

## UNITED STATES PATENT OFFICE

2,058,237

## LUBRICANT

Gus Kaufman and Oney P. Puryear, Beacon,  
N. Y., assignors to The Texas Company, New  
York, N. Y., a corporation of Delaware

No Drawing. Application March 21, 1934,  
Serial No. 716,649

9 Claims. (Cl. 87—9)

This invention relates to lubricants and has to do particularly with the manufacture of greases for lubricating ball and roller bearings.

An object of the invention is to provide a grease for the lubrication of ball and roller bearings, such as those of modern high speed and low power machinery, which will not change appreciably in texture and consistency under the heat and rapid agitation encountered in service.

Another object of the invention is to prepare a grease that possesses low starting and running torques and causes no appreciable drag on the moving parts.

A further object of the invention is to manufacture a grease suitable as a protective coating for bearings while in storage and that is strongly resistant to oxidation whereby no gum is formed which will stick or damage the bearings.

Further objects of the invention will be observed from the following description and examples of the invention.

The greases used heretofore, such as the soda soap greases of fatty oils like tallow oil, in order to lubricate at low temperatures, must be made so soft or of such low melting points that they run off the bearings at high temperatures while if they are made sufficiently hard or of such high melting points to lubricate at high temperatures they become spongy and exert an excessive drag on the machinery, or the bearings form channels therein and fail to receive adequate lubrication.

We have now discovered how to produce greases which meet the practical requirements of present day ball and roller bearing machinery. We have found that the product obtained by proper oxidation of paraffin wax is a desirable constituent of such greases. However, in the use of this material it is necessary to combine it in proper proportions with other materials, as will be explained hereinafter.

The oxidized paraffin wax, which may be used advantageously according to the present invention is produced by such controlled oxidation that the product has a high ratio of saponification to acid value and is characterized by its freedom from gummy materials insoluble in hydrocarbon oils. Products particularly suitable for use are described in U. S. Patent No. 1,668,871, May 8, 1928, to Joseph R. Scanlin, and U. S. Patent No. 1,909,945, May 23, 1933, to Benjamin Gallsworthy. We prefer to use the sweatings from oxidized paraffin wax, as described in the Gallsworthy patent.

In the preparation of our improved greases we saponify the sweatings from the oxidized paraffin wax and then mix the resulting soap with a suitable quantity of hydrocarbon lubricating oil to give the proper consistency. While the greases produced as just described function satisfactorily as ball and roller bearing lubricants it is sometimes advantageous, particularly to improve their

coherence and consistency, to incorporate with the foregoing greases a suitable amount of one or more other soaps. We have found that the addition of the soda soaps of naphthenic or stearic acids is often beneficial and aids substantially in the realization of the desired grease.

The following examples illustrate practical methods of preparing our improved lubricants in accordance with the invention.

|                                      | 10    | Per cent |
|--------------------------------------|-------|----------|
| Sweatings from oxidized paraffin wax | 28.53 |          |
| Caustic soda (43% aqueous solution)  | 6.42  |          |
| Pale oil (300 viscosity at 100° F.)  | 36.52 | 15       |
| Water                                | 28.53 |          |

A sample of oxidized paraffin wax prepared substantially in accordance with the foregoing Gallsworthy patent was sweated at 90°—100° F. and separated into approximately two-thirds of semi-liquid sweatings and one-third solid waxy material. The sweatings so obtained had approximately the following tests: gravity, 25.5° Bé.; viscosity, 305 seconds; Saybolt at 100° F.; pour, 95° F.; neutralization number, 25.8; and saponification number, 129.

A portion (10 lbs.) of the sweatings was charged to a grease kettle equipped with mechanical agitation and heated to 165° F. when a 43% aqueous solution (2½ lbs.) of caustic soda and water (10 lbs.) were added. The mixture was slowly heated with agitation to a temperature of 260° F. during a period of about 10 hours. Pale oil (12.8 lbs.) of 300 viscosity Saybolt Universal at 100° F. was then slowly added over a period of about 1½ hours. The grease was cooled to about 200° F. and drawn from the kettle. The product had a smooth buttery texture resembling heavy petroleum. The grease tested as follows:

|                                                   |         |    |
|---------------------------------------------------|---------|----|
| Sodium soap                                       | 16.3%   |    |
| Alcohol soluble                                   | 11.6%   |    |
| Water soluble and alcohol insoluble               | 4.7%    |    |
| Oils                                              | 80.4%   | 45 |
| Water                                             | 2.4%    |    |
| Free alkali (as Na <sub>2</sub> CO <sub>3</sub> ) | 1.7%    |    |
| A. S. T. M. penetration:                          |         |    |
| Unworked                                          | 185     |    |
| Worked                                            | 305     | 50 |
| Melting point                                     | 260° F. |    |

The finished product lubricated satisfactorily on ball and roller bearings up to 320° F.

|                                     | 55    | Per cent |
|-------------------------------------|-------|----------|
| Naphthenic acids                    | 35.26 |          |
| Pale oil (300 viscosity at 100° F.) | 52.51 |          |
| Caustic soda (43% aqueous solution) | 7.30  |          |
| Water                               | 4.93  | 60       |

A sample (14.3 lbs.) of naphthenic acids of 116 saponification value was charged to a grease kettle and heated to 105° F. and then a 43% aqueous solution (2.96 lbs.) of caustic soda and water 5 (2 lbs.) were added. The mixture was agitated and heated over a period of about 6 hours to 236° F. The product began to thicken and 300 pale lubricating oil (21.3 lbs.) was slowly added and the mixture heated to 262° F. during about 10 4 hours. The grease was cooled to 212° F. and drawn from the kettle. The resultant product tested as follows:

|                         |            |
|-------------------------|------------|
| Sodium naphthenate      | 26.1%      |
| Free alkali             | 0.45%      |
| Mineral oil             | 72.1%      |
| Water                   | Trace      |
| A. S. T. M. penetration | Too liquid |
| Melting point           | 160° F.    |

20 *Example 3*

Per cent

|                     |    |
|---------------------|----|
| Grease of Example 1 | 50 |
| Grease of Example 2 | 50 |

25 Equal proportions of the naphthenic acid soap grease of Example 2 and the oxidized paraffin wax grease of Example 1 were charged to a grease kettle. The mixture was heated and stirred for about 2 hours while the temperature rose to 30 290° F. The resulting product had a melting point of 182° F. and an A. S. T. M. penetration of 30 286. The calculated analysis of the grease was 30 as follows:

|                                      |       |
|--------------------------------------|-------|
| Per cent                             |       |
| Sodium soap of oxidized paraffin wax | 8.15  |
| Sodium soap of naphthenic acids      | 13.05 |
| Oils                                 | 77.92 |
| Free alkali (as NaOH)                | 0.88  |

40 The grease gave excellent results when used as 40 a lubricant for ball and roller bearings at operating temperatures up to 320° F. and a speed of about 1725 R. P. M.

45 *Example 4*

Per cent

|                                        |       |
|----------------------------------------|-------|
| Stearic acid                           | 12.78 |
| Caustic soda (43% aqueous solution)    | 4.42  |
| Pale oil (90-100 viscosity at 210° F.) | 82.80 |

50 Stearic acid (10 lbs.) and 90-100 viscosity at 210° F. pale oil (9.5 lbs.) were charged to a grease kettle, agitated and heated to about 228° F. A 43% aqueous solution of caustic soda (3.46 lbs.) was then added during an interval of about 1 hour. The remainder of the mineral oil (55.3 lbs.) was slowly added during about 4 hours while the temperature was raised sufficiently to boil off the water. The maximum temperature was 55 263° F. The product was cooled to 186° F. and drawn from the kettle. The resulting grease had a good body, was smooth and glossy and somewhat stringy. In actual test it lubricated well at low temperatures but it thickened and became 60 spongy at about 250° F., and ran off the bearings at about 280° F. It tested as follows:

|                         |         |
|-------------------------|---------|
| Sodium soap             | 13.41%  |
| Free alkali             | 0.03%   |
| Oils                    | 85.30%  |
| Water                   | None    |
| A. S. T. M. penetration | 331     |
| Melting point           | 365° F. |

Example 5

Per cent

|                     |    |
|---------------------|----|
| Grease of Example 1 | 50 |
| Grease of Example 4 | 50 |

Equal proportions of the sodium stearate soap grease of Example 4 and the sodium soap of oxidized paraffin wax grease of Example 1 were charged to a grease kettle and agitated for about 2 hours while the mixture was slowly heated to 5 about 255° F. The product was cooled to 180° F. and drawn from the kettle. The resulting grease had a smooth and uniform texture. It gave excellent lubrication on ball and roller bearings at temperatures of 320° F. The tests on the 10 product were as follows:

|                          |         |
|--------------------------|---------|
| Sodium soap (calculated) | 14.86%  |
| Free alkali              | 0.69%   |
| Water                    | 1.00%   |
| Oils (by difference)     | 83.45%  |
| A. S. T. M. penetration  | 167     |
| Melting point            | 338° F. |

Although we have described three specific greases (Examples 1, 3 and 5) which are satisfactory, we do not intend that they should limit the scope of our invention. Thus we may vary considerably the proportions of the soap and mineral oil in the greases. In case the grease is made from oxidized paraffin wax soap alone and mineral oil, the soap may vary from 10-25% with good results. In Example 3, we have shown the ratio of oxidized paraffin wax soap to naphthenic acid soap in the grease to be about 1:2. This ratio may vary within the limits of about 2:1 and 1:2 with good results. It is also not necessary to use 30 300 pale oil since any good grade of lubricating oil varying in viscosity from about 200 at 100° F. to about 100 at 210° F. Saybolt Universal may be used. In general about 70-85% of mineral oil is satisfactory.

Obviously many modifications and variations of the invention, as hereinbefore set forth, may be made without departing from the spirit and scope thereof, and therefore only such limitations should be imposed as are indicated in the appended claims.

We claim:

1. A lubricating grease having about the following percentage composition:

|                                                                                         |      |
|-----------------------------------------------------------------------------------------|------|
| Per cent                                                                                |      |
| Soda soap of oxidized paraffin wax sweatings                                            | 16.3 |
| Hydrocarbon lubricating oil (Saybolt viscosity in excess of about 200 secs. at 100° F.) | 50   |
| Water                                                                                   | 2.4  |
| Free alkali                                                                             | 1.7  |

2. A lubricating grease for ball and roller bearings having about the following percentage composition:

|                                                                                         |       |
|-----------------------------------------------------------------------------------------|-------|
| Per cent                                                                                |       |
| Soda soap of sweatings from oxidized paraffin wax                                       | 8.15  |
| Soda soap of naphthenic acids                                                           | 13.05 |
| Hydrocarbon lubricating oil (Saybolt viscosity in excess of about 200 secs. at 100° F.) | 77.92 |
| Free alkali                                                                             | 0.88  |

3. A lubricating grease for ball and roller bearings having about the following percentage composition:

|                                                   |       |
|---------------------------------------------------|-------|
| Per cent                                          |       |
| Soda soap of sweatings from oxidized paraffin wax | 8.15  |
| Soda soap of stearic acid                         | 6.71  |
| Hydrocarbon oil                                   | 83.45 |
| Water                                             | 1.00  |
| Free alkali                                       | 0.69  |

4. A lubricating grease consisting essentially of about 10-25% of soda soap of oxidized paraffin wax and hydrocarbon lubricating oil, said oxidized wax having a high ratio of saponification to acid value and being substantially free from gummy materials, said grease being substantially free from saponifiable constituents and having a high melting point and the characteristics when applied to ball and roller bearing lubrication of low starting and running torques and sufficient consistency when hot to be retained on said bearings at a temperature in the region of 320° F.

5. A lubricating grease consisting essentially of about 16% of soda soap of oxidized paraffin wax sweatings and hydrocarbon lubricating oil, said oxidized paraffin wax sweatings having a high ratio of saponification to acid value and being substantially free from gummy materials, said grease being substantially free from saponifiable constituents and having a high melting point and the characteristics when applied to ball and roller bearing lubrication of low starting and running torques and sufficient consistency when hot to be retained on said bearings at a temperature in the region of 320° F.

6. A lubricating grease consisting essentially of mixed alkali metal soaps of oxidized paraffin wax and naphthenic acids, and 70-85% of hydrocarbon lubricating oil, the ratio of soap of oxidized paraffin wax to soap of naphthenic acids being between the ratios of 1:2 and 2:1, said oxidized paraffin wax having a high ratio of saponification to acid value and being substantially free from gummy materials, said grease being substantially free from saponifiable constituents and having a high melting point and the characteristics of low starting and running torques and sufficient consistency when hot to be retained on said bearings at a temperature in the region of 320° F.

7. A lubricating grease consisting essentially of mixed soda-soaps of oxidized paraffin wax sweatings and naphthenic acids, and in the region of

80% of hydrocarbon lubricating oil, the ratio of soap of oxidized paraffin wax sweatings to soap of naphthenic acids being about 1:2, said oxidized paraffin wax sweatings having a high ratio of saponification to acid value and being substantially free from gummy materials, said grease being substantially free from saponifiable constituents and having a high melting point and the characteristics when applied to ball and roller bearing lubrication of low starting and running torques and sufficient consistency when hot to be retained on said bearings at a temperature in the region of 320° F.

8. A lubricating grease consisting essentially of mixed soda-soaps of oxidized paraffin wax and stearic acid, in about equal proportions, and about 70-85% of hydrocarbon lubricating oil, said oxidized paraffin wax having a high ratio of saponification to acid value and being substantially free from gummy materials, said grease being substantially free from saponifiable constituents and having a high melting point and the characteristics when applied to ball and roller bearing lubrication of low starting and running torques and sufficient consistency when hot to be retained on said bearings at a temperature in the region of 320° F.

9. A lubricating grease consisting essentially of about 15% of mixed soaps of oxidized paraffin wax sweatings and stearic acid, in about equal proportions, and hydrocarbon lubricating oil, said oxidized paraffin wax sweatings having a high ratio of saponification to acid value and being substantially free from gummy materials, said grease being substantially free from saponifiable constituents and having a high melting point and the characteristics when applied to ball and roller bearing lubrication of low starting and running torques and sufficient consistency when hot to be retained on said bearings at a temperature in the region of 320° F.

GUS KAUFMAN.  
ONEY P. PURYEAR.